

## UNITED STATES PATENT OFFICE.

WILLIAM WITTE, OF PROVIDENCE, RHODE ISLAND, ASSIGNOR TO THE UNITED STATES FINISHING COMPANY, OF NEW YORK, N. Y., A CORPORATION OF CONNECTICUT.

## PROCESS OF FINISHING FABRICS AND TO THE FABRIC AND COMPOSITION.

No Drawing.

Application filed June 29, 1926. Serial No. 119,472.

This invention relates to a process of finishing cloth, and more particularly to the process of treating reformed by regenerated cellulose fibres to remove the lustre, and to the fabric and composition.

The manufacture of the artificial silk is commonly conducted from cellulose by first rendering the cellulose soluble by forming a soluble cellulose-substitution product, then 10 forming the substitution product into the requisite fine fibres, and subsequently removing the substituted radicals to reform the cellulose. Such a product may be termed a reformed cellulose, and bears the trade name 15 of viscose fibres. It has a fine texture and high lustre comparable to silk. Such a fibre, however, while it may be used to imitate lustrous silk fabrics, has not heretofore been capable of satisfactory manufacture into 20 lustreless fabrics.

It is an object of this invention to treat viscose fibres to remove the lustre while retaining the softness and strength.

For many purposes, moreover, it is desirable to form a fabric with varied patterns, including portions having lustre and portions devoid of lustre. Such fabrics may be made by combining in a Jacquard loom 25 fibres which in themselves are lustrous with those which are not. Such manufacture, however, is so expensive that it is, for many purposes, prohibitive.

It is a further object of this invention, therefore, to devise a method for removing 35 the lustre from such fibres, which is adapted to a printing process, so that the gloss can be removed from a woven fabric in any printed pattern desired.

It has furthermore been found that such 40 viscose fibre, when delusterized, possesses other physical properties which are advantageous.

The deglossing operation in accordance 45 with this invention is apparently an operation of changing the exterior surface of the individual viscose fibres into a substitution product devoid of lustre, but the complexity of the cellulose molecules is such that it is difficult to determine just what substitution 50 has taken place.

This invention finds the most useful application in the production of a damask effect upon viscose fabrics by printing. It will therefore be here illustrated as specifically carried out in a printing operation.

One such practical method of carrying out the process is as follows:

There is a mixed solution of a suitable alcohol such as 90% ethyl alcohol and 10% caustic soda to form an alcohol-caustic solution. This is then mixed with a suitable thickening agent and solvent—a practical mixture being 50 grams of the alcohol-caustic solution, 25 grams of gum sandarac, 24 grams of ethyl alcohol, and one gram of 60 pyridene. The use of the gum renders the composition viscous and suitable for printing, and it is desirable where the printing compound is in itself not sufficiently viscous.

The composition may then be printed upon the fabric in the same manner that dye-stuffs are printed. The fabric is then preferably dried to prevent spreading of the design, although satisfactory results can be obtained without drying, if care be taken in 70 the manipulation. The results of the above step are believed to be the formation of an alkali substitution product of the substance of the fibres, although in all probability this reaction is a surface action only.

The fabric so treated may then be subjected to a bath capable of effecting the final substitution. A bath suitable for this purpose may be formed by dissolving in carbon-tetrachloride, 10% to 25% of para-toluene-85 sulpho-chloride. This bath is preferably used at a temperature of from 100 to 150 degrees F., and the fabric need be subjected thereto only for a short period. It is then wrung out and rinsed in a 5% soda ash solution and subsequently in a 5% soap solution, both at approximately 180 degrees F., until it is free from odor and from the reagents of the prior baths.

By the above treatment it will be found 95 that those portions of the cloth on which the caustic-alcohol solution was printed have lost the lustre, but maintain their softness and strength.

Since certain changes may be made in 100 carrying out the above process without departing from the scope of the invention, it is intended that all matter contained in the above description shall be interpreted as illustrative and not in a limiting sense.

It is also to be understood that the following claims are intended to cover all of the generic and specific features of the invention herein described, and all statements of the scope of the invention which, as a matter 110

of language, might be said to fall therebetween.

Having described my invention, what I claim as new and desire to secure by Letters 5 Patent, is:

1. The process of treating viscose fibres to remove lustre which comprises treating the alkalinized fibre with para-toluene-sulphochloride.
- 10 2. The process of treating viscose fabrics to remove lustre which comprises applying to the fabric a chemical having a thick and gummy consistency, and capable of effecting a substitution product, and thereafter subjecting the entire fabric to a second substitution process to form a lustreless substitution product from the first mentioned substitution product.
- 15 3. The process of treating a viscose fibre which comprises applying a viscous composition capable of forming a substitution product, thereafter subjecting the fibre to a bath capable of forming a second substitution product from the first, which bath is not a solvent for the first mentioned composition.

4. The process of figuring fabrics which comprises printing thereon a substance capable of altering the chemical composition of the fibre, subjecting the same to a second 30 bath in which the printed substance is insoluble and capable of effecting an alteration of the composition resulting from said first mentioned alteration and subsequently removing all uncombined treatment chemicals. 35

5. A process of forming a pattern upon viscose fabrics which comprises effecting a substitution in the molecule by a printing compound and subsequently effecting a second substitution by immersion.

6. A printing compound for removing lustre from viscose fabrics comprising an alcohol-caustic solution thickened with gum.

7. The process of forming a pattern upon viscose fabrics, which comprises reacting upon the same by two chemicals which, together, are capable of effecting lustreless substitution in the molecules, including the application of one of said chemicals by printing.

In testimony whereof I affix my signature.

WILLIAM WITTE.